

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## PROCESS OF PRODUCING WHITE WOOD PULP FOR HIGH GRADE PAPER MANUFACTURE

No Drawing.

Application filed May 16, 1931. Serial No. 537,997.

This invention relates to a process of producing an improved wood pulp more especially from kraft pulp, and possessing not only the important papermaking characteristics, including strength and tear resistance, 5 of the kraft pulp from which it is derived, but further possessing a pure white color and far greater freedom from resins and ash content and a notably lower pentosan content than its derivation material. The product 10 produced by the process of the present invention is thus one which fulfills the desiderata in two fields of papermaking, namely, that devoted to the manufacture of bond, ledger, 15 and writing papers, wherein whiteness of fiber is a prime desideratum, and that devoted to the manufacture of envelope, bag papers, and the like, wherein strength and tear resistance, as well as whiteness of fiber, are 20 highly prized.

Those skilled in the art well know that the conversion of kraft pulp to whiteness is a difficult task, which when accomplished by the use of a hypochlorite bleach liquor is accompanied 25 both by exceedingly high bleach usage and marked injury to the papermaking characteristics of the fiber. The process of the present invention, however, is aimed at the preservation of the valuable papermaking 30 characteristics of kraft pulp while removing from such pulp so much of its coloring matter and other constituents as are undesirable from a papermaker's standpoint. The process of the present invention does not 35 result in a product which is of extraordinarily high alpha cellulose content, for if it be attempted to refine kraft pulp markedly in so far as concerns increasing its alpha cellulose content, it loses especially in such properties as strength, even though it may be improved in other respects, such as softness and 40 stability.

In practising the process of the present invention, I proceed as follows. A raw kraft 45 pulp is subjected to the action of chlorine water or to hypochlorite bleach liquor, or to a succession of such reagents, without visible whitening of the pulp. In fact, the chlorine and/or hypochlorite should be used in such 50 amount that the pulp after treatment has a

distinctly different hue than the raw kraft pulp. For example, raw pulp may be treated at temperatures of from 50° to 100° F. for two to six hours, as a 4% to 6% stock suspension in chlorine water containing 4% to 8% 55 chlorine, based on pulp. During this treatment, the pulp assumes a deep orange color. The treated pulp is then washed free of treating reagent and reaction products. When the washed pulp is tested, it exhibits a lower 60 lignin content than that present in the original pulp. Ligneous matter is thus removed from the pulp without injury to its papermaking characteristics. The prechlorinated stock may be antichlored or neutralized, if 65 desired, to remove residual chlorine before it is subjected to a washing operation.

The washed pulp is then treated with an alkaline liquor preferably similar to the cooking liquor used in the kraft process of fiber liberation, namely, one containing both caustic soda and sodium sulphide. Preferably, the liquor is one containing 2% to 4% alkali, calculated as caustic soda equivalent, but 40% of which alkali is present in the form 70 of sodium sulphide. The pulp is suspended in this specific liquor as an 8% to 10% stock suspension at about 40° to 70° C., for from about one to four hours. During this treatment, the pulp is further freed from lignous 75 matter, but without impairing its paper marking characteristics. The pulp is then washed, at which stage it has a lignin content of from 80 1% to 2.5%, as against a lignin content of from 3% to 7% in the raw kraft pulp. It is 85 thus seen that the process thus far is directed largely at the selective removal from the pulp of lignous matter, the initial treatment selectively removing some of the lignin and chlorinating the rest, and the second treatment being conducted in an alkaline solution under conditions to dissolve out the chlorinated lignous matter. The selective dissolving 90 out of the chlorinated lignous matter, as already indicated, takes place at particular temperature conditions in a solution containing particular amounts of both caustic soda and sodium sulphide. Such temperature conditions are conducive to the desired dissolving out action without the marked refin- 95 100

ing effect on the fiber which might be accomplished at higher temperatures or with a higher concentration of alkali in solution. For instance, if the treatment of the pulp be carried out at higher temperature with the solution of alkali hereinbefore described, say 90° to 100° C. or higher, it is found that there is a marked sacrifice in the tear resistance of the pulp, even though its Mullen or pop strength is not appreciably affected. On the other hand, if the treatment of the pulp be carried out at temperatures lower than those specified with the solution of alkali hereinbefore described, there is a less effective removal of lignin from the pulp and a strong tendency to reduce the Mullen and tensile strength of the pulp; and there is apt to be an increase in the alpha cellulose content of the pulp to a point where it approaches the softness and other characteristics of a refined wood pulp. It is thus seen that the treatment of the pulp with a solution of alkali to produce the desired product is conducted, in accordance with the present invention, within a temperature and alkalinity range designed to effect an extensive elimination of lignin from the pulp without appreciably affecting its alpha cellulose content or its strength and tear resistance characteristics. In this connection, it is to be observed that alkaline liquors other than that mentioned may be used, so long as the conditions of alkalinity and temperature of the liquor are such as will remove largely residual ligneous reaction products from the pulp, as a result of the initial treatment of the pulp with an oxidant, while substantially preserving the alpha cellulose content of the pulp. For instance, another alkali, such as sodium carbonate, may be used in lieu of caustic soda in an alkaline liquor of about 4% alkali content, calculated as caustic soda equivalent, about 40% of which alkali may be present in the form of sodium sulphide. The temperature of digestion in such case should be about 70° C. to effect the desired removal of ligneous matter in a reasonably short period of time. Such an alkaline liquor, containing sodium carbonate and of about 40% sulphidity, is available in a kraft mill, as a result of the recovery operations practised therein. Thus, the smelted inorganic residuum issuing from the smelting furnace of a kraft mill consists essentially only of sodium carbonate and sodium sulphide, the sodium sulphide content of the smelt ranging from as low as about 20% to as high as about 40%. The smelt may be dissolved in water, and, after filtration, may be adjusted in alkali content for use in treating kraft pulp which has undergone an initial treatment with oxidant as hereinbefore described. If desired, the alkaline liquor may be a straight sodium carbonate solution of the strength hereinbefore indicated containing a small amount of sodium hypochlorite bleach, say 2% to 3%, based

on the weight of pulp. The presence of this amount of bleach does not perceptibly affect the strength of the pulp, but does facilitate subsequent bleaching of the pulp to whiteness. It may further be mentioned that the alkaline treatment may be effected in two stages, first with comparatively dilute solution of such alkalies as lime or sodium carbonate at elevated temperatures, and then with the stronger and more expensive alkaline solutions at lower temperatures as has been described in detail, the initial alkaline treatment serving to eliminate from the pulp essentially only the easily removable chlorination reaction products. 70

The alkaline-digested and washed pulp is now ready to be bleached. Bleaching, too, must be carried out in a special way, in order to arrive at my novel product. To this end, the pulp is preferably subjected to a series of three independent bleaching treatments. The first two bleaching treatments consist in maintaining the pulp for three to six hours as a 5% suspension in hypochlorite bleach liquors at 70° F.,—about 3% calcium hypochlorite based on pulp being used in the first treatment, about 2% calcium hypochlorite based on pulp being used in the second treatment, and about 0.5% caustic soda based on pulp being added to the bleaching liquors in each treatment. The pulp is washed and thickened between the first two treatments, and again washed and thickened after the second treatment. The third and final bleaching treatment may consist in treating the pulp with sufficient bleach, rendered alkaline throughout the bleaching operation by the presence of free alkali, to produce a product of pure whiteness, but other bleaching agents, such as peroxides, permanganates, and perborates may be used in this final bleaching treatment. At the end of this treatment, the pulp is washed, but when permanganates are used, it has a light tan color because of residual manganese oxides clinging to the fiber. The oxides may be completely removed by treating the pulp with a dilute sulphurous acid or bisulphite solution and washing. 80

The resulting product, which is in pure-white condition, may be delivered to machines which form sheets ready for shipment. The bleaching treatments described effect a whitening of the pulp substantially without injury to the physical or papermaking characteristics thereof, but the degree of whiteness attained is of course subject to some variation. In fact, the final bleaching treatment or one of the intermediate bleaching treatments may be omitted to produce a pulp possessing a fair degree of whiteness. Indeed, the succession of bleaching treatments and alternate washings preserve the physical characteristics of the pulp while converting it to a white condition; and the final bleach- 85 90 95 100 105 110 115 120 125 130

ing treatment is conducted when the pulp is nearly pure white, and so requires such a dilute solution of bleaching agent as to acquire pure whiteness with no observable physical degradation.

The following table indicates the transformation effected upon the given kraft pulp in practising the process of the present invention:

|                            | Kraft     | Product of the process of present invention |
|----------------------------|-----------|---------------------------------------------|
| Color                      | Brown.    | Pure white.                                 |
| Total cellulose (per cent) | 90 - 93.0 | 98.5 - 99.5                                 |
| Alpha cellulose (per cent) | 89        | 87 - 89                                     |
| Cu. No.                    | 1.2       | 1.0 - 2.0                                   |
| Ash (per cent)             | .6 - 1.0  | 0.1 - 0.3                                   |
| Resins (per cent)          | .2 - .4   | 0.1 - 0.3                                   |
| Pentosans (per cent)       | .7 - .9   | 3.0 - 5.0                                   |
| Strength                   | 150 - 160 | 150 - 160                                   |
| Tear resistance            | 250 - 270 | 250 - 270                                   |

It is to be observed that the product produced by the process of the present invention, in addition to having the papermaking characteristics, including strength and tear resistance, of kraft pulp, is of pure-white color and has an extremely low resin content,—in fact being lower in resinous specks than most bleached sulphite pulps on the market. It has a much higher total cellulose content than the original pulp, but its alpha cellulose content is practically the same as that of the original pulp. Its pentosan content is somewhat lower than that of the original pulp, but there are sufficient pentosans therein in a form imparting toughness or strength to the sheet, without developing the brittleness imparted to a kraft pulp when it is whitened, for example, by successive treatments with sulphurous acid and hypochlorite bleach liquor.

While the product has been described as being produced more especially from kraft pulp, it may be prepared by my process from other suitable alkaline-cooked wood pulps, for instance, the long-fibered soda pulps obtained by effecting fiber liberation from coniferous woods in so-called soda cooking liquors.

I do not herein claim the novel product resulting from the process of the present invention, as such a product has been described and claimed in my application Ser. No. 496,566, filed November 18, 1930, now Patent No. 1,809,287, dated June 9, 1931. So far as subject matter is concerned, this application is a continuation in part of my application Serial No. 189,461, filed May 6, 1927, and Serial No. 292,325, filed July 12, 1928.

What I claim is:

1. A process which comprises treating unbleached, alkaline-cooked wood pulp with an oxidant of the character of chlorine or hypochlorite to react upon lignous groups in such pulp, digesting the pulp at about 40° to 70° C. in an alkaline liquor containing about 2%

to 4% alkali, calculated as caustic soda equivalent, to remove largely lignous reaction products from such pulp while substantially preserving unchanged the alpha cellulose content of such pulp, and bleaching the digested pulp to whiteness while substantially preserving its physical characteristics.

2. A process which comprises treating unbleached, alkaline-cooked wood pulp with an oxidant of the character of chlorine or hypochlorite to react upon lignous groups in such pulp, digesting the pulp at about 40° to 70° C. in an alkaline liquor containing about 2% to 4% alkali, calculated as caustic soda equivalent but in the form of caustic soda and a sodium sulphide, to remove largely lignous reaction products from such pulp while substantially preserving unchanged the alpha cellulose content of such pulp, and bleaching the digested pulp to whiteness while substantially preserving its physical characteristics.

3. A process which comprises treating unbleached, alkaline-cooked wood pulp with an oxidant of the character of chlorine or hypochlorite to react upon lignous groups in such pulp, digesting the pulp at about 40° to 70° C. in an alkaline liquor containing about 2% to 4% alkali, calculated as caustic soda equivalent but in the form of sodium carbonate and sodium sulphide, to remove largely lignous reaction products from such pulp while substantially preserving unchanged the alpha cellulose content of such pulp, and bleaching the digested pulp to whiteness while substantially preserving its physical characteristics.

4. A process which comprises treating unbleached, alkaline-cooked wood pulp with chlorine water containing 4% to 8% chlorine, based on pulp, until the chlorine is substantially consumed, digesting the chlorinated pulp for about one to four hours at about 40° to 70° C. in an alkaline liquor containing about 2% to 4% alkali, calculated as caustic soda equivalent, to remove largely lignous reaction products from such pulp while substantially preserving unchanged the alpha cellulose content of such pulp, and bleaching the digested pulp to whiteness while substantially preserving its physical characteristics.

5. A process which comprises treating unbleached, alkaline-cooked wood pulp with an oxidant of the character of chlorine or hypochlorite to react upon lignous groups in such pulp, digesting the pulp in an alkaline liquor under conditions of alkalinity and temperature of liquor correlated with time of digestion to remove largely lignous reaction products from such pulp while substantially preserving unchanged the alpha cellulose content of such pulp, and subjecting the digested pulp to more than one bath of distinctly alkaline hypochlorite bleaching liquor under conditions to preserve the physical characteristics of such pulp substantially unimpaired.

6. A process which comprises treating un-  
bleached, alkaline-cooked wood pulp with an  
oxidant of the character of chlorine or hypo-  
chlorite to react upon ligneous groups in such  
5 pulp, digesting the pulp in an alkaline liquor  
under conditions of alkalinity and tempera-  
ture of liquor correlated with time of diges-  
tion to remove largely ligneous reaction prod-  
ucts from such pulp while substantially pre-  
10 serving unchanged the alpha cellulose con-  
tent of such pulp, and subjecting the digested  
pulp to more than one distinctly alkaline  
hypochlorite bleaching treatment and alter-  
nate washings under conditions to preserve  
15 the physical characteristics of such pulp sub-  
stantially unimpaired.

In testimony whereof I have affixed my  
signature.

GEORGE A. RICHTER.

20

25

30

35

40

45

50

55

60

65